

Sept. 24, 1940.

H. F. BAUER

2,215,848

PREPARATION OF PREGUMMED HANGING PAPER

Filed April 19, 1939



INVENTOR.  
*Harold Bauer*  
BY *Richard Spencer*  
ATTORNEY.

## UNITED STATES PATENT OFFICE

2,215,848

## PREPARATION OF PREGUMMED HANGING PAPER

Hans F. Bauer, Chicago, Ill., assignor to Stein, Hall Manufacturing Company, Chicago, Ill., a corporation of Delaware

Application April 19, 1939, Serial No. 268,780

10 Claims. (Cl. 91—68)

This invention relates to pregummed hanging papers, more particularly wall papers, poster papers, bill board papers and the like, having a dried coating of adhesive thereon which requires only moistening to be applied to a wall or other surface.

Wall papers and other types of hanging papers, including poster papers and bill board papers, are ordinarily applied to a wall or other surface by a paper hanger who makes up a paste and puts it onto the paper just before applying the paper to the wall or other surface. It has heretofore been proposed to make wall papers having a self-contained adhesive, but these papers have generally been unsatisfactory because of the numerous problems involved. Thus, Lobdell, Reissue Patent No. 10,430 described a wall paper which is dry sized on its back and according to the patent may be hanged by moistening the sized surface and applying it to a wall. The sizing used is said to be dextrine, glue, paste or gums.

No practical or suitable pregummed hanging paper has ever resulted from the teaching of the Lobdell patent because the problem of making a pregummed hanging paper is not so simple that it may be done merely by adding an ordinary type of sizing material or glue to the back of the paper and drying it. A pregummed hanging paper such as a pregummed wall paper must have certain characteristics which cannot be obtained with an ordinary adhesive. For instance, it must be flexible, non-curling and the adhesive must not crack or chip off of the paper. The adhesive must be spread uniformly on the paper and when applied to the wall must dry and shrink evenly so as to shrink out any blisters or bulges which form on the surface of the paper. In view of the numerous problems involved, little progress has heretofore been made in the preparation of pregummed hanging papers or more specifically, in the preparation of pregummed wall papers.

In my copending application, Serial No. 252,457, filed January 23, 1939 now matured into U. S. Patent No. 2,183,532, which in turn is a continuation-in-part of my application Serial No. 168,360 filed October 11, 1937, I have described a new and improved type of pregummed hanging paper. The adhesive on said paper comprises a plurality of amylaceous substances of differing water absorptive capacities and a plasticizing agent having the property of increasing the fluidity of amylaceous dispersions.

One of the objects of the present invention is to provide an improved type of pregummed hang-

ing paper without the necessity of using a plurality of amylaceous substances to form the dried coating on the back of the paper. Other objects of the invention will appear hereinafter.

It has now been found in accordance with the invention that a pregummed hanging paper may be made by using a specified type of degraded or modified amylaceous substance in forming the adhesive coating for the back of the paper. This degraded or modified amylaceous substance for the purpose of this invention should have a solubility within the range of about .5% to about 30% in water at 75° F. and when mixed with proportions of water in the ratio of 10 parts of water to 1 part of amylaceous material should have a fluidity or viscosity characteristic within the range of 7 seconds to 200 seconds, as determined by the following test on a Stormer viscosimeter.

This test involves determining the number of seconds required for 100 revolutions of the viscosimeter cup containing a given sample of material at 75° F., using a 100 gram weight. The sample of amylaceous material to be tested is made up by heating 1 part of said material in 10 parts of water to a temperature of 185° F. until a homogeneous dispersion is obtained, then cooling to 75° F. The viscosimeter cylinder used in testing the amylaceous substances hereinafter referred to required 2.8 seconds for 100 revolutions running free, using a 100 gram weight, and 5.9 seconds with water at 75° F. This test is herein referred to as the "viscosity test for degraded amylaceous substances."

In practicing the invention, it has been found that amylaceous degradation products of the character described when dispersed with a plasticizing agent capable of increasing the fluidity of aqueous amylaceous dispersions are excellent adhesives for the manufacture of pregummed hanging papers. Pregummed hanging papers made up with adhesive compositions of this type have sufficient adhesive power to adhere to plane surfaces when the adhesive coating is moistened. At the same time they have excellent slip characteristics and may be moved from one point to another after the dried coating of adhesive is remoistened while the adhesive is still wet and after it is first applied to a surface. Furthermore, blisters, bulges, wrinkles and the like which sometimes form when a hanging paper such as a wall paper is applied in the wet state shrink out or disappear in pregummed hanging papers of the type herein described as the paper dries. Another important feature of the pregummed hanging papers made in accordance with this in-

vention is to be found in the fact that the dried adhesive coating does not tend to become tacky and cause the paper to stick together when rolled in the usual manner, nor does the adhesive coating tend to crack or cause the paper to curl when it is properly applied to the paper.

For the purpose of this invention, it is preferable that the total solid content of the adhesive before it is applied to the paper or other base material be such that not less than about 1 part of water and not more than about 5 parts of water per part of solids is required to give a viscosity within the range of about 40 seconds to about 180 seconds at 75° F. using a 1000 gram weight in the above mentioned viscosity test instead of a 100 gram weight. This test is referred to herein as the "adhesive composition" viscosity test. By total solids content is meant the amyloseous material plus plasticizing agents and any other normally solid materials that may be employed.

The ratio of solids to water should preferably not be less than about 1:1 using an amyloseous degradation product of the type herein referred to, or otherwise the adhesive character of the coating will not be sufficient upon remoistening to give the required slip characteristics. On the other hand, if the ratio of water to solids is greater than about 5:1, the amount of drying required in order to properly apply the adhesive to the paper or other material which is to be coated will normally be prohibitive.

In the coating operation the coating weight is always important because it determines the amount of adhesive material actually on the paper. If this amount is too great, it may cause the adhesive to crack or check. If it is too small, the adhesive will not have the necessary strength to hold the paper on the wall or other surface to which it is applied. Generally speaking, for the purpose of this invention the amount of water required will preferably be about 2 to 3 parts of water per part of solids in order to apply the adhesive to the paper or other base material at a suitable or proper coating weight.

The plasticizing agent preferably employed in accordance with this invention in order to prepare the adhesive is a normally solid substance or a plurality of normally solid substances that exert a solubilizing influence on amyloseous materials. The term "amyloseous materials" is used herein to describe starch and starch degradation products. "Degraded amyloseous materials" or "amyloseous degradation products" as the expressions are used herein, cover dextrinized starches and modified starches. A dextrinized starch is a starch which has been converted either in the wet or dry state in the presence of an acid or an acid reacting substance. If converted in the dry state, it is referred to herein as a dry converted dextrinized starch. A modified starch is a starch which generally retains its starch structure but has been chemically treated or treated in some other manner, for example, by means of enzymes, so as to break down or modify this starch structure. For example, chlorinated starches and thin boiling starches may be called modified starches.

A raw or undegraded starch alone is unsuitable for the purpose of this invention for several reasons, one of which is to be found in the fact that this type of starch requires too much water for the proper dispersion. On the other hand, certain types of starch degradation products, as for

example, those containing relatively large amounts of dextrin are also unsuitable for use alone in the preparation of pregummed hanging papers in accordance with this invention, largely due to the fact that these products are too tacky when formed into a dried coating and then remoistened. The result is that a pregummed hanging paper made from such materials does not have the necessary slip characteristics.

The adhesive which is used in preparing the pregummed hanging material is prepared by dispersing the ingredients, namely, the degraded amyloseous substance, plasticizing agents and any other auxiliary materials in a dispersion medium such as water in sufficient amount to give the mixture a fluidity corresponding to that mentioned above so that it may be suitably spread or coated upon the paper. The resultant composition is then applied to the paper by any suitable method of surface coating involving the use of a doctor blade or other means such as are well known to those skilled in the coating art, and the paper is then dried or allowed to dry. The coating weight will vary depending upon the composition of the adhesive, the speed and method of applying, and also upon the type of material treated. With ordinary wall papers good results may be obtained by the use of 2 grams or less (e.g., say about 1.2 grams) of adhesive per square foot of wall paper, calculated on the weight of the dried adhesive coating. For some base materials, as low as 0.5 gram of dried adhesive per square foot may be used while for others it may be desirable to use as high as 5 grams per square foot. Relatively heavy papers, for example, on the order of 12 ounce papers or more, are preferred, but the invention is not limited in this respect, as anyone skilled in the coating art can vary the quantity of adhesive within relatively wide ranges to obtain an adhesive coating suited to the particular type of paper and to the use to which the paper is to be put.

Other features and advantages of the invention will be apparent by reference to the following specification and the accompanying drawing, in which the single figure represents wall paper having a self-contained adhesive, as herein described.

As illustrated in the drawing, the wall paper, which may be of any suitable character or design, has a self-contained adhesive backing 2, as more fully hereinafter described.

The invention will be further illustrated but is not limited by the following examples in which the quantities are stated in parts by weight unless otherwise indicated.

#### Example 1

A starch conversion product was prepared by converting a high grade wheat starch for 1 hour at 280° F. This conversion was carried out in a substantially dry state, using 2½ lbs. of 18° Bé. hydrochloric acid to 1000 lbs. of wheat starch. The acid was diluted to 6° Bé. before being added to the wheat starch. After being converted 1 hour at 280° F. the conversion product was removed and was found to be 6.4% soluble in water at 75° F. This product when tested at 75° F. with 10 parts of water per part of said product on a Stormer viscosimeter using a 100 gram weight in the manner previously described gave a viscosity test of 11 seconds in 100 revolutions of the viscosimeter cylinder.

The conversion product thus prepared was

mixed with a composition having the following ingredients:

|                           | Parts |
|---------------------------|-------|
| Urea                      | 25    |
| 5 Sodium acetate          | 10    |
| 75% sulfonated castor oil | 1.75  |

These ingredients were blended together dry and then mixed with the starch conversion product in the ratio of 35 lbs. to 65 lbs. of the conversion product. The resultant blend was then blended with 1 1/4 parts of water per part of blend and this mixture was heated to 185° F. until clear.

It was coated on the back of wall paper in a thin film which was allowed to dry. Wall paper thus prepared was non-curling, non-cracking, flexible and the adhesive was non-tacky under ordinary atmospheric conditions. When this adhesive is moistened, the paper possesses excellent slip characteristics so that it will slide from one place to another after it has been applied to a wall and before the adhesive has dried substantially. At the same time, it possesses sufficient retack power to hold it to the wall. Blisters, wrinkles and the like which sometimes form in the paper when it is applied readily shrink out when the paper dries on the wall.

In this example the amount of sodium acetate may be increased to 15% or decreased to 5%, the amount of urea being correspondingly decreased or increased.

#### Example II

A wheat starch conversion product was prepared from a lower grade wheat starch known as No. 25, the conversion conditions being otherwise the same as for the wheat starch conversion in Example I. This conversion product had a solubility of 2.6% in water at 75° F. and a Stormer viscosity as determined in the manner previously described at 75° F., with a 100 gram weight of 17.2 seconds in 100 revolutions of the cylinder. Sixty-five parts of this conversion product were blended with 35 parts of a plasticizing composition made up of 25 parts urea, 10 parts sodium acetate and 1 1/4 parts of 75% sulfonated castor oil. This blend was then mixed with 2 parts of water per part of blend and the mixture heated while stirring to 185° F. until clear. The resultant composition had a viscosity characteristic of 72 seconds as determined on a Stormer viscosimeter at 75° F. using a 1000 gram weight for 100 revolutions of the cylinder.

This adhesive composition when applied to the back of wall paper to form a pregummed wall paper gave excellent results similar to those described in Example I.

#### Example III

The procedure in this example was the same as in Example I except that the starch conversion product was made from a low grade wheat starch known as No. 50. This conversion product had a solubility of 4.4% at 75° F. and a Stormer viscosity in 10 parts of water per part of said product at 75° F. of 19 seconds using a 100 gram weight according to the test previously described.

A blend of 65 lbs. of this product with 35 lbs. of a plasticizing composition containing 25% urea, 10% sodium acetate and 1 1/4% of 75% sulfonated castor oil when mixed with 2 1/2 parts of water per part of blend and heated to 185° F. until clear gave an excellent adhesive composition for the preparation of pregummed hanging paper. This adhesive composition at 75° F. using a 1000 gram weight with a Stormer viscosimeter gave a fluid-

ity or viscosity corresponding to 70 seconds for 100 revolutions of the viscosimeter cylinder.

Excellent results were obtained when this composition was employed to form pregummed hanging paper.

#### Example IV

In Example I, the conversion product was obtained from practically 100% pure wheat starch from which substantially all of the gluten had been removed. In Example II, the conversion product was obtained from a somewhat lower grade of wheat starch, which in Example III a still lower grade of wheat starch was used containing gluten in dispersed form. According to the present example the material used as a starting material was wheat flour in which the gluten was rendered inert by the following conversions: This was converted for 1 hour with sodium bisulfite using about 2 lbs. of sodium bi-sulfite to 1200 lbs. of flour at a temperature of about 225° F., then there was added 50 lbs. of boric acid and 3 lbs. of 18° Bé. hydrochloric acid diluted to 6° Bé. hydrochloric acid and the temperature was raised to 280° F. for 1 1/2 hours to 2 hours more. The conversion product obtained had a solubility within the range of 8% to 12% at about 75° F. and gave a Stormer viscosity test in 10 parts of water per part of said product when tested with a 100 gram weight in the manner previously described of 14 seconds at 75° F.

This conversion product also formed an excellent adhesive for the preparation of pregummed hanging paper when mixed with about 4 parts of water per part of conversion product and blended with urea and sodium acetate in the proportion of about 65 parts of conversion product, 25 parts of urea and 10 parts sodium acetate with the addition of about 1 1/4 parts of 75% sulfonated castor oil.

#### Example V

A rice starch conversion product was prepared by adding to 1000 lbs. of rice 3 lbs. of 18° Bé. hydrochloric acid which was diluted to 6° Bé. and converted at 280° F. for about 2 1/2 hours. This conversion product had a solubility of 1% in water at about 75° F. and gave a Stormer viscosity test in 10 parts of water per part of conversion product of 29.5 seconds using a 100 gram weight according to the test procedure previously described.

This conversion product was blended with urea, sodium acetate and sulfonated castor oil in the proportions of 65 parts conversion product, 25 parts urea, 10 parts sodium acetate and 1 1/4 parts 75% sulfonated castor oil and the blend mixed with water in proportions of 3 parts of water to 1 part of blend and heated to 185° F. until clear. The resultant composition gave a viscosity test on a Stormer viscosimeter of 97 seconds using a 1000 gram weight for 100 revolutions of the cylinder at 75° F.

Excellent results were obtained in the preparation of pregummed hanging papers with this adhesive composition.

#### Example VI

Similarly good results were obtained using a rice starch conversion product prepared as in Example V except that the time of conversion was 3 1/2 hours and the solubility was 1.6% in water at 75° F. The Stormer viscosity of this conversion product using 10 parts of water per part of conversion product and a 100 gram weight at 75° F. according to the procedure previously described was about 23 seconds.

This conversion product was mixed with a plasticizing composition containing 25 parts urea, 10 parts sodium acetate and 1 1/4 parts of 75% sulfonated castor oil, the proportions of plasticizing agent to conversion product being 35 lbs. to 65 lbs. The resultant blend when mixed with 3 parts of water per part of blend and heated to 180° F. formed an excellent adhesive for the manufacture of pregummed hanging materials 10 and had a viscosity of 70 seconds as determined on a Stormer viscosimeter for 100 revolutions of the viscosimeter cylinder using a 1000 gram weight at 75° F.

*Example VII*

15 A rice starch conversion product was formed according to the general methods of Examples V and VI except that the time of conversion was 4 1/2 hours and the conversion product had a solubility of 9.2% at 75° F. with a viscosity characteristic of 8.5 seconds when tested with 10 parts of water per part of conversion product on a Stormer viscosimeter at 75° F. in the manner previously described. This product was blended with a plasticizing composition made up of 25 parts 20 urea, 10 parts sodium acetate, and 1 1/4 parts of sulfonated castor oil, the proportions being such that the total blend consisted of 65% rice conversion product and 35% of the plasticizing composition. This blend was then mixed with 1 1/2 25 parts of water per part of blend and heated to 185° F. This composition showed a viscosity characteristic of 106 seconds as determined on a Stormer viscosimeter for 100 revolutions of the viscosimeter cylinder at 75° F. using a 1000 gram weight.

30 Excellent results were obtained with this composition in the preparation of pregummed hanging papers of various types including wall paper, poster paper, bill board paper, etc.

40 *Example VIII*

In this example the degraded amylose substance employed was a No. 90 thin boiling starch, a type of starch well known in the trade, made 45 by the wet conversion of corn. This starch had a solubility in water at 75° F. of about 15% and a fluidity or viscosity characteristic of 10.5 seconds when tested on a Stormer viscosimeter in 10 parts of water per part of starch at 75° F. according to the test previously given. Sixty-five 50 lbs. of this starch were blended with 35 lbs. of a plasticizing composition made up of 25 parts urea, 10 parts sodium acetate and 1 1/4 parts sulfonated castor oil. This blend was then mixed with 1 1/2 55 parts water per part of blend and heated to 185° F. The resultant adhesive composition had a viscosity characteristic of 70 seconds when tested on a Stormer viscosimeter at 75° F. using a 1000 gram weight. Good results were obtained in the 60 use of this composition for the preparation of pregummed wall paper.

*Example IX*

A chlorinated starch sold under the trade name 65 of Hercules and having a solubility of 1.8% in water at 75° F. and a Stormer viscosity of 11.2 seconds when tested in 10 parts of water to 1 part of starch at 75° F., according to the method previously given, was blended with a plasticizing 70 composition in the ratio of 65% of starch to 35% of the plasticizing composition. This plasticizing composition contained 25 parts urea, 10 parts sodium acetate and 1 1/4 parts sulfonated castor oil. The blend, when mixed with 1 1/2 parts of 75 water per part of blend and heated to 185° F.

gave an adhesive composition which on cooling to 75° F. and testing in a Stormer viscosimeter had a fluidity or viscosity characteristic of 89 seconds for 100 revolutions of the viscosimeter cylinder using a 1000 gram weight. Good results were obtained in the use of this composition for the preparation of pregummed wall paper.

*Example X*

10 In this example, the conversion product was a corn starch conversion product having a solubility of about 4.2% and a Stormer viscosity characteristic of 16 seconds at 75° F. when tested with 10 parts of water per part of conversion 15 product according to the viscosity test for degraded amylose substances previously described. This conversion product was blended with a plasticizing composition to produce a blend containing 65% conversion product and 35% of the plasticizing composition. The plasticizing composition contained 25 parts urea, 10 parts sodium acetate and 1 1/4 parts 75% sulfonated castor oil. This blend was then mixed with 1 1/4 parts water per part of blend and heated to 185° 20 F. until clear. The resultant composition had a viscosity or a fluidity characteristic of 70 seconds when tested on a Stormer viscosimeter at 75° F. using a 1000 gram weight.

25 This product also is suitable for use in the preparation of pregummed hanging papers.

30 In a similar manner other types of degraded amylose substances may be employed for the preparation of pregummed hanging papers provided they fall within the general range of solubilities and viscosity previously mentioned. For 35 example, a No. 75 thin boiling starch can be employed which has a solubility of about .8% in water at about 75° F. and a Stormer viscosity of about 193.5 seconds when tested in 10 parts of water per part of starch according to the test 40 herein given using a 1000 gram weight. This starch degradation product starch represents approximately the starchiest type of material which can be used as the sole amylose substance in order to obtain suitable results for the purpose of 45 the present invention. Thus, a number 60 thin boiling starch is too starchy in its nature and requires too much water in order to be practical for the purpose of this invention. On the other hand, certain types of dextrines having a solubility of say 75% to 80% or more contain too much dextrose and do not have the proper solubility and fluidity or viscosity characteristics for the preparation of a pregummed wall paper as 50 provided by this invention. Thus, it will be seen 55 that the invention is confined to a specific range of amylose degradation products. It will be understood of course that these products may be blended with other types of amylose products or other materials than those specifically described herein, but the advantage of the present invention is to be found mainly in the fact that it is no longer necessary to use a blend of 60 amylose materials.

This invention is not limited to any particular 65 type of amylose degradation product and the starch materials from which these products are derived may be, for example, wheat, rice, barley, corn, rye, tapioca, potato and other types of starches. In carrying out this invention, however, it has been found that certain types of starch degradation products within the limits defined give outstanding results as compared 70 with others. Among the starch degradation products which are particularly desirable are 75

those derived from wheat and rice because these conversion products within the limits defined herein form softer pastes which do not tend to gel as distinguished, for example, from certain 5 other grain starches, such as corn, which can be used although it is less desirable. With wheat and rice starches, the preferred amylaceous degradation products have a solubility within the range of about 1% to about 25% and a viscosity 10 characteristic within the range of about 8 seconds to about 30 seconds, as determined by the viscosity test for degraded amylaceous substances herein described. Likewise, degraded tuber starches such as tapioca and potato within 15 the defined limits can be used but are less desirable because the adhesives made from them are tackier than the grain starch degradation products. This tackiness is offset to a considerable extent by salts of aliphatic carboxylic acids such as sodium acetate which imparts slip to 20 the adhesive.

It will be understood that variations may be made in the composition of the adhesive, in the method of applying the adhesive to the base 25 material and in the various types of base materials to which it is applied. Many wall papers are unsized or contain very little sizing, while poster papers and bill board papers are often highly sized and the type of adhesive within the 30 range specified herein may vary depending upon the sizing and other factors related to the use of a particular base material.

The plasticizing agent employed is preferably a normally solid material which has the property 35 of increasing the fluidity of dispersions of degraded amylaceous substances. Urea and alkali metal acetates both have this property and in the examples the urea may be used without the alkali metal acetate, or vice versa, but the combination 40 of both appears to give results which are more than merely additive. Furthermore, the combination of both together apparently tends to prevent curling of the paper. Urea is practically neutral in aqueous solution and 45 sodium acetate in water ordinarily has a pH from 7 to 8 so that neither compound is injurious to the paper. Urea and/or sodium acetate may be replaced at least in part by other substances which are not injurious to the paper and which 50 have a solubilizing or dispersing action on starch degradation products, as, for example, the water soluble analogues and homologues of urea, including thiourea, other alkali metal acetates such as potassium acetate, other salts of aliphatic 55 carboxylic acids such as sodium propionate and other propionates, and many other materials such, for example, as resorcinol, chloral hydrate, sodium salicylate, calcium chloride, zinc chloride, magnesium chloride, water soluble thiocyanates, including potassium thiocyanate, sodium thiocyanate and ammonium thiocyanate, and water soluble nitrates, including sodium nitrate, potassium nitrate, ammonium nitrate and guanidine nitrate. Some compounds such as those 60 of phenolic nature, however, sometimes suffer from the disadvantage that they tend to turn dark. The compound or compounds chosen should preferably be normally solid at ordinary temperatures since the presence of a liquid compound might tend to make the paper stick together when rolled. It is also preferable that the compound chosen be such that the pH value of the adhesive under the conditions used can be within the range of about 5 to about 9. Bleaching 65 agents may be added, for example, sodium

bisulfite or sodium hydrosulfite. Fillers may also be used to give body to the adhesive composition.

If either the urea or sodium acetate is omitted, the proportion of the ingredient retained is preferably correspondingly increased. In addition to its advantages in preventing curling of the paper, sodium acetate also produced a clear film and tends to prevent crystallization of urea in the film so that the final appearance of the paper is such that the adhesive is not readily visible to 10 the casual observer.

The amount of solubilizing or dispersing agent, as already indicated, should preferably be such that the composition will spread evenly and uniformly upon the addition of about 1 to about 5 parts of water per part of blended solid ingredients. The presence of too much urea is to be avoided because of a tendency to make the composition hygroscopic. This tendency is less marked with sodium acetate. Generally speaking, of the total solids content, a major portion should be formed by the amylaceous degradation product and the total amount of plasticizing composition should not be greater than about 20 45% of the total solids. Thus, the total amount of urea and sodium acetate is preferably not greater than about 45% of the total solids preferably within the range of 20% to 45%. The minimum amount of sodium acetate is preferably 25 about 5% and the maximum about 30% of the total solids. The minimum amount of urea is preferably about 5% and the maximum about 40% of the total solids.

In some instances it may be desirable to add an 35 acid, preferably in amounts just sufficient to neutralize any ammonia which may be formed. For this purpose very small quantities of acid are required, being in the neighborhood of around 2% or less. Acids which are normally 40 solid at ordinary temperatures are preferred, for example, citric acid, tartaric acid, malic acid, boric acid and the like.

The sodium acetate employed may be granular or powdered sodium acetate, either 60%, 90% or 45 anhydrous, the first mentioned being preferred. Sodium diacetate having available acetic acid of from 25% to 35% may also be used.

The mixing of the various ingredients of the adhesive compositions and the temperature of 50 heating may vary, but ordinarily it will be sufficient to heat the mixture within the range of about 140° F. to about 185° F. until a uniform homogeneous dispersion is obtained.

The expression "water soluble urea" as employed herein is intended to include and cover urea and its water soluble analogues and homologues, including thiourea, monomethyl urea, monoethyl urea, dimethyl urea and higher water soluble homologues or analogues which have the 60 property of increasing the fluidity of aqueous amylaceous dispersions. The expression "lower aliphatic carboxylic acid" is intended to cover members of the fatty acid series which are substantially soluble in water.

The pregummed hanging papers made in accordance with this invention upon being moistened have the desired slip characteristics for application to walls and other plane surfaces. This invention makes possible the preparation of 70 pregummed hanging papers in a simpler manner than it has heretofore been possible to make such materials. At the same time, this is accomplished while producing pregummed hanging papers having all of the desirable characteristics 75

of freedom from tack and stickiness in the dry state, freedom from cracking, checking and curling. The amount of water present initially in the adhesive when it is applied to the paper is 5 such that it does not tend to destroy the paper. Moreover, the adhesive is weakly acid, substantially neutral or mildly alkaline, and the ingredients thereof do not tend to injure the paper or the wall to which the paper is applied. The 10 adhesive, furthermore, does not tend to lose its adhesive characteristics over long periods of time, that is to say, the adhesive retains its remoistening adhesive properties when a dried coating thereof is moistened with water, even though the 15 dried coating had been allowed to stand for a considerable length of time, as would be the case with wall papers or other wall coverings which are not sold immediately.

It will be understood that variations may be 20 made in the composition of the adhesive and in the paper or other base material to which it is applied without departing from the invention, and that in carrying out the invention, other variations, modifications and equivalents may be 25 employed. Thus, the base material, instead of being paper, may be a canvas wall covering, or a thin wooden panel, or some other type of fibrous wall covering in which proper slip characteristics of the adhesive are essential to match patterns. 30 Reference is hereby made to my co-pending application Serial No. 184,929, filed January 14, 1938, now matured into United States Patent No. 2,183,736, which covers certain new and improved adhesive compositions including some of 35 the compositions which may be employed for making pregummed hanging papers, as set forth in my United States Patent No. 2,183,532, previously referred to and in which the adhesive comprises a plurality of amylaceous substances of differing water absorptive capacities, at least one of which has a relatively high water absorptive capacity and another a relatively low water absorptive capacity.

Having thus described the invention, what I 45 claim as new and desire to secure by Letters Patent of the United States is:

1. A pregummed wall paper having a dried coating of adhesive thereon formed from an incompletely dextrinized wheat starch having a 50 solubility in water at 75° F. from about 1% to about 25% and a viscosity characteristic within the range of about 8 seconds to about 30 seconds as determined by the viscosity test for degraded amylaceous substances herein described, intimately dispersed with urea and sodium acetate, the dextrinized wheat starch forming a major part of the adhesive, the total amount of urea and sodium acetate being about 20% to about 45% by weight of the total solids, the minimum 55 and maximum amounts of sodium acetate being about 5% and about 30%, respectively, and the minimum and maximum amounts of urea being about 5% and 40%, respectively, on the basis of the total solids, said adhesive also containing a 60 small amount of sulfonated oil on the basis of the normally solid ingredients.

2. A pregummed wall paper having a dried coating of adhesive thereon formed from an incompletely dextrinized wheat starch having a 65 solubility in water at 75° F. from about 1% to 25% and a viscosity characteristic within the range of about 8 seconds to about 30 seconds, as determined by the viscosity test for degraded amylaceous substances herein described, intimately dispersed with urea and an alkali metal

acetate, the dextrinized wheat starch forming a major part of the adhesive, the total amount of urea and alkali metal acetate being about 20% to 45% by weight of the total solids, the minimum and maximum amounts of alkali metal acetate being about 5% and about 30%, respectively, and the minimum and maximum amounts of urea being about 5% and about 40%, respectively, on the basis of total solids.

3. A pregummed hanging paper having a dried coating of adhesive thereon formed from an incompletely dextrinized wheat starch having a solubility in water at 75° F. from about 1% to about 25% and a viscosity characteristic within the range of about 8 seconds to about 30 seconds, as determined by the viscosity test for degraded amylaceous substances herein described, intimately dispersed with a water soluble urea and an alkali metal acetate, the total amount of the urea and alkali metal acetate being not more than about 45% by weight of the total solids, the minimum and maximum amounts of alkali metal acetate being about 5% and about 30%, respectively, and the minimum and maximum amounts of urea being about 5% and about 40%, respectively, on the basis of the total solids, said ingredients being present in such proportions that said adhesive coating when moistened possesses retack properties and slip characteristics permitting said material to slide after it has first been moistened and while the adhesive is still wet and after it is first applied to a surface.

4. A pregummed wall covering having a dried coating of adhesive thereon formed from an incompletely dextrinized rice starch having a solubility in water at 75° F. from about 1% to about 25% and a viscosity characteristic within the range of about 8 seconds to 30 seconds, as determined by the viscosity test for degraded amylaceous substances herein described, intimately dispersed with a water soluble urea and an alkali metal acetate, the total amount of the urea and alkali metal acetate being about 20% to about 45% by weight of the total solids, the minimum and maximum amounts of alkali metal acetate being about 5% and about 30%, respectively, and the minimum and maximum amounts of the urea being about 5% and about 40%, respectively, on the basis of the total solids.

5. A pregummed hanging paper having a dried coating of adhesive thereon formed from a degraded grain starch having a solubility in water at 75° F. within the range of about .5% to about 30%, and a viscosity characteristic within the range of about 7 seconds to 200 seconds, as determined by the viscosity test for degraded amylaceous substances herein described, intimately dispersed with a water soluble urea and an alkali metal acetate, the total amount of the urea and the alkali metal acetate being not more than about 45% by weight of the total solids, the minimum and maximum amounts of alkali metal acetate being about 5% and about 30%, respectively, and the minimum and maximum amounts of the urea being about 5% and about 40%, respectively, on the basis of the total solids, said ingredients being present in such proportions that said adhesive coating when moistened possesses retack properties and slip characteristics permitting said material to slide while the adhesive is still wet after it is first applied to a surface.

6. A pregummed hanging paper having a dried coating of adhesive thereon formed from a degraded amylaceous substance having a solubility

5

15

20

25

30

35

40

45

50

55

60

65

70

75

in water at 75° F. from about .5% to about 30% and a viscosity characteristic within the range of about 7 to about 200 seconds, as determined by the viscosity test for degraded amyloseous substance herein described, intimately dispersed with a water soluble urea and a soluble salt of a lower aliphatic carboxylic acid, the total amount of the urea and said salt being not more than about 45% by weight of the total solids, the minimum and maximum amounts of said salt being about 5% and about 30%, respectively, and the minimum and maximum amounts of the urea being about 5% and about 40%, respectively, on the basis of total solids, said ingredients being present in such proportions that said adhesive coating when moistened possesses retack properties sufficient to hold said paper against a surface to which it is applied and slip characteristics permitting said material to slide against said surface while it is still wet after it is first applied to said surface.

7. A pregummed hanging paper having a dried coating of adhesive thereon formed from a degraded amyloseous substance having a solubility in water at 75° F. from about .5% to about 30% and a viscosity characteristic within the range of about 7 seconds to about 200 seconds, as determined by the viscosity test for degraded amyloseous substances herein described, intimately dispersed with a substantially neutral, normally solid compound of such character that it will not injure the paper and having a solubilizing action on said degraded amyloseous substance and an alkali metal acetate, said ingredients being present in such proportions that said adhesive-coating when moistened possesses retack properties and slip characteristics permitting said paper to slide while the adhesive is still wet and after it is first applied to a surface.

8. A pregummed hanging paper having a dried coating of adhesive thereon formed from a degraded amyloseous substance having a solubility in water at 75° F. within the range of about .5% to about 30% and a viscosity characteristic within the range of about 7 seconds to about 200 seconds, as determined by the viscosity test for degraded amyloseous substances herein described, intimately associated with at least one normally solid compound of such character that it will not injure the paper and having a solubilizing action on degraded amyloseous substances, the propor-

tions of said ingredients being such as to produce an adhesive coating which after being dried is capable of being remoistened and possesses retack properties and slip characteristics permitting the paper to be moved after paper containing the adhesive has been moistened and first applied to a plane surface while the adhesive is still wet.

9. A pregummed hanging material comprising a flexible sheet material having thereon a dried coating of an adhesive formed from a degraded amyloseous substance having a solubility in water at 75° F. from about .5% to about 30% and a viscosity characteristic within the range of about 7 seconds to about 200 seconds, as determined by the viscosity test for degraded amyloseous substances herein described, intimately dispersed and associated with at least one plasticizing agent which is noninjurious to the base material and has the property of increasing the fluidity of aqueous amyloseous compositions, said adhesive having a pH within the range from about 5 to about 9, and said ingredients being present in such proportions that said adhesive coating when moistened possesses retack properties sufficient to cause the sheet material to adhere to a plane surface while permitting said material to slide on said surface while the adhesive is still wet after it is first applied.

10. A pregummed hanging material comprising a base material having thereon a dried coating of an adhesive formed from a degraded amyloseous substance having a solubility in water at 75° F. from about .5% to about 30% and a viscosity characteristic within the range of 7 seconds to about 200 seconds as determined by the viscosity test for degraded amyloseous substances herein described, intimately dispersed and associated with at least one plasticizing agent which is non-injurious to the base material and has the property of increasing the fluidity of dispersions of degraded amyloseous substances, said ingredients being present in such proportions that said adhesive coating when moistened possesses retack properties and slip characteristics permitting said material to slide while the adhesive is still wet after it is first applied to a surface.

HANS F. BAUER.